

June 21, 1960

J. N. MASON

2,941,913

ELASTOMERIC FLOOR COVERING

Filed May 31, 1957

3 Sheets-Sheet 1



June 21, 1960

J. N. MASON

2,941,913

ELASTOMERIC FLOOR COVERING

Filed May 31, 1957

3 Sheets-Sheet 2



Fig. 3

INVENTOR

James N. Mason  
BY  
Kenny, Jenny, Walter, Billieh

ATTORNEYS

June 21, 1960

J. N. MASON

2,941,913

ELASTOMERIC FLOOR COVERING

Filed May 31, 1957

3 Sheets-Sheet 3



Fig. 4

INVENTOR

James N. Mason

BY

Kennedy, Jenney, Water, Hilliard

ATTORNEYS

2,941,913

## ELASTOMERIC FLOOR COVERING

James N. Mason, Winchester, Mass., assignor to Boston Woven Hose and Rubber Company, Cambridge, Mass., a corporation of Massachusetts

Filed May 31, 1957, Ser. No. 662,768

2 Claims. (Cl. 154—49)

This invention comprises a new and improved elastomeric floor covering, using that term to mean floor covering of natural or synthetic rubber as well as plastic composition.

Many types of this elastomeric floor covering are molded with special surface contours and with special decorative designs in color imprinted on the exposed surface of the flooring prior to molding. The finished product is a flooring with a predetermined colored surface pattern and a distinct surface texture modifying the appearance of the flooring by scattering reflected light in different directions.

Such floorings are usually made by printing a homogeneous base stock of desired thickness with a decorative surface pattern of inks, colored latices, or plastic compositions having different colors from the base stock. Since the base stock is ordinarily not completely covered by the overlying pattern, the color of the base stock shows as an additional surface color and this may be made to contribute to the pattern. For certain uses the base stock may be substantially obscured by the colored inks of the printed or sprayed pattern and in such flooring the base stock is usually of much cheaper material than the pattern inks.

In the actual use of floorings made as above described, a serious problem has arisen due to the fact that the surface pattern stocks are thin and tend to wear through on the ridges or raised portions of the surface contour. The worn areas thus occurring allow the base color to show as a wear pattern, thereby partially destroying the original contrastingly colored surface pattern and radically impairing the appearance of the flooring in the worn area. This objectionable change in appearance greatly reduces the service life of the product and decreases its value.

I have discovered that these objections may be obviated and other advantages achieved by establishing a novel relation between the base stock, the colored decorative pattern, and the surface configuration or texture of the flooring. For example, in flooring having a molded contour pattern of ridges or corrugations, or at least of elongated raised portions which may take the form of regularly arranged ridges, the wear pattern resulting from the wearing away of the tops of these ridges will then consist of more or less straight or long oval areas having the color of the exposed base stock. In accordance with the present invention it is now proposed to imprint on the surface of the flooring a colored pattern which is carefully designed to include areas resembling both in color, size and eye effect the worn areas which will subsequently be developed due to ordinary wear of the flooring. These special areas of the imprinted design may consist of irregular elongated lines, or areas of special shapes, which coincide with the areas normally developed on the particular surface contour of the covering due to wear, that is to say, the ridge or rib areas.

In one aspect the elastomeric flooring of this invention may be described as presenting a corrugated wearing surface and including in its structure an underlying ply of elastomeric material of uniform color and an overlying

colored ornamental surface design thereon including in its pattern a multiplicity of lines coinciding in location and direction with the crests of the corrugations and being of the same color as the underlying base ply.

For example, the underlying ply may be of a dark color and the decorative surface layer of lighter color, but including at least one color similar to that of the darker base stock, or the arrangement may be reversed and the underlying ply may be of a light color and the surface layer mainly of darker colors in the valleys and light color on the ridges.

These and other features of the invention will be best understood and appreciated from the following description of one embodiment thereof selected for purposes of illustration and shown in the accompanying drawings in which:

Fig. 1 is a plan view of flooring having a typical print pattern,

Fig. 2 is a corresponding view in cross section on an enlarged scale, showing the pattern layer as worn from the crests of the corrugations,

Fig. 3 is a plan view of the wear pattern, and

Fig. 4 is a view of the flooring of Fig. 1 after it has been subjected to wear.

The floor covering shown in Figs. 1 and 2 comprises an underlying body 8 of solid dark colored elastomeric material molded to present in its upper surface a series of uniformly spaced parallel corrugations. A typical rubber-type composition is the following:

|    |                                            |
|----|--------------------------------------------|
| 30 | 5.00 pounds weight of smoked sheets        |
|    | 40.00 pounds weight of whole tire reclaim  |
|    | 5.00 pounds weight of mineral rubber       |
|    | 1.25 pounds weight of zinc oxide           |
|    | 8.00 pounds weight of furnace carbon black |
| 35 | .30 pound weight of mercaptobenzothiazole  |
|    | .10 pound weight of diphenylguanidine      |
|    | .50 pound weight of stearic acid           |
|    | .50 pound weight of paraffine wax          |
|    | 2.00 pounds weight of sulfur               |
| 40 | 37.35 pounds weight of calcium carbonate   |
|    | 100.00 pounds total                        |

A typical plastic-type composition is as follows:

|    |                                         |
|----|-----------------------------------------|
| 45 | 100 pounds weight of polyvinyl chloride |
|    | 25 pounds weight of dioctylphthalate    |
|    | 10 pounds weight of tricresylphosphate  |
|    | 125 pounds weight of calcium carbonate  |
|    | 1 pound weight of stearic acid          |
| 50 | 5 pounds weight of basic lead carbonate |
|    | 1 pound weight of carbon black          |

267 pounds total

Prior to the molding operation an ornamental surface pattern is applied to the upper face of the base stock by printing with inks, latex emulsions, or plastic compositions or in any convenient manner. The decorative surface layer applied in this manner may be relatively thin, for example not be over .01" in thickness and its material may be considerably more expensive than the composition of the underlying base stock. The ornamented base stock is now bonded to a thick layer of inexpensive bottom stock 8 and molded therewith to form longitudinal corrugations or ridges 9. In general the applied pattern will be distinguished by the portions applied and contained in the valleys between the ribs or ridges 9 of the flooring in contrast with the base color appearing upon the crest of the ribs after extensive wear has occurred.

When the ribbed flooring of Fig. 1 is subjected to wear, it develops a wear pattern like that suggested in Fig. 3, that is to say, the decorative surface material is

worn from the crests of the ribs in some such areas as those indicated by the dark streaks in Fig. 3. This has been established empirically and depends on the location receiving the wear and the texture and wear-resisting characteristics of the material in those particular areas.

Fig. 4 represents the appearance of the partially worn matting and is derived from superposing the wear pattern of Fig. 3 upon the unworn pattern of Fig. 1. The effect of wear is to uncover or enlarge areas of base color in the material of the base stock, and on account of the arrangement and disposition of the pattern this increase in the visible base color areas does not result in any conspicuous alteration in the original ornamental pattern. This is apparent from a comparison of Figs. 1 and 4. As an illustration of the actual inconspicuous change in the appearance of the pattern, attention is called to the areas 10 and 11 in Fig. 1, the worn area 12 in Fig. 3, and the superposed effect of the area 12 shown in combination with the areas 10 and 11 in Fig. 4. Similar differences between the unworn and worn patterns may be detected on close examination of Figs. 1 and 4, but it is strikingly apparent that the general effect of the worn and unworn patterns is substantially unchanged to the observer.

This application is a continuation-in-part of my co-pending application Ser. No. 507,570, filed May 11, 1955, now abandoned in favor of the present application.

Having thus disclosed my invention and described in detail a preferred embodiment thereof, I claim as new and desire to secure by Letters Patent:

1. A new type of elastomeric flooring presenting a corrugated wearing surface and including an underlying 30

thin surface layer substantially entirely covering said underlying ply not more than 0.01" in thickness and of a lighter color displayed in an ornamental pattern including discontinuous darker lines corresponding in color to said underlying ply and extending generally lengthwise of the crests of the corrugated wearing surface, whereby the ornamental pattern of the flooring will remain substantially unchanged when the crests of the thin surface layer have been removed by wear.

2. A new type of elastomeric flooring presenting a corrugated wearing surface and including an underlying ply of elastomeric material of a uniform base color, and a thin surface layer superimposed above and substantially covering said underlying ply, not more than about 0.01" in thickness, the surface layer presenting various different colors displayed in an ornamental pattern including discontinuous areas corresponding in color to the color of said underlying ply and extending generally upon and in the direction of the crests of the corrugated wearing surface, whereby the ornamental pattern of the flooring will remain substantially unchanged when the crests of the surface layer have been removed by wear.

#### References Cited in the file of this patent

#### UNITED STATES PATENTS

|           |                |               |
|-----------|----------------|---------------|
| 1,751,546 | Glidden et al. | Mar. 25, 1930 |
| 1,985,480 | Carpenter      | Dec. 25, 1934 |
| 1,989,703 | Leguillon      | Feb. 5, 1935  |
| 1,989,704 | Leguillon      | Feb. 5, 1935  |
| 2,243,736 | Loblein        | May 27, 1941  |
| 2,818,824 | Read et al.    | Jan. 7, 1958  |